

1

3,592,633  
**HIGH STRENGTH LOW ALLOY STEEL POSSESSING SUFFICIENT WELDABILITY CONTAINING SMALL AMOUNTS OF Nb, Ti, AND B**  
Tatsumi Osuka, Junichi Tanaka, Michio Hayashida, and Yoshiaki Ono, Kawasaki-shi, Japan, assignors to Nippon Kokan Kabushiki Kaisha  
No Drawing. Filed Jan. 22, 1969, Ser. No. 802,715  
Claims priority, application Japan, Jan. 22, 1968,  
43/3,389  
Int. Cl. C22c 37/10, 39/02  
U.S. Cl. 75—124

4 Claims

**ABSTRACT OF THE DISCLOSURE**

High-strength low-alloy steel keeping yield strength of more than 70 kg./mm.<sup>2</sup> in a further coordinated relationship with specific small amounts of alloying ingredients, particularly Nb+Ti+B, and possessing good toughness and sufficient weldability through an ordinary quench-temper heat-treatment.

The present invention relates to high strength low alloy steels and, more particularly, to high strength steels for welding structural services.

It is well-known that many high-strength low alloy steels having yield points of more than 70 kg./mm.<sup>2</sup> are employed widely or welding structural services. In such cases, both high strength and superior toughness are generally required. These characteristics were obtained by adding a considerable amount of alloying elements with ordinary quench-temper heat treatment. Such conditions of alloying elements, however, make hardenability of steels increase and are apt to bring about cracks at welding zone of steels. For elimination of said defects, pre-heating of more than 100° C. is generally required. The higher the pre-heating temperatures, the higher the cost becomes. Difficulties of such temperature control increase also in the field of welding steels.

It has now been discovered that by maintaining specified and coordinated ranges of alloying elements, the above defects can be completely eliminated. According to the present invention, the low carbon steel possesses a yield point of more than 70 kg./mm.<sup>2</sup> and superior toughness and has been proved in reduced hardenability in welding and decreased crack sensitivity.

It is an object of the present invention to provide a novel high strength low alloy steel, particularly containing 0.005% to 0.04% Nb, 0.0005% to 0.005% B and 0.005% to 0.05% Ti.

Other objects and advantages will become apparent from the following descriptions and illustrative examples. The invention also contemplates providing a unique steel particularly adapted to be employed in the welding structure.

Generally speaking, the present invention contemplates the manufacture of steels heat-treated with quenching of adapting liquids (containing water), gases (containing air), or mixtures of above media at a temperature from AC<sub>3</sub> point to 1050° C. and then with tempering at a temperature of less than AC<sub>1</sub> point.

The steels of the present invention are composed of the following constituents:

2

|            | Percent by weight |
|------------|-------------------|
| C          | 0.05-0.15         |
| Si         | 0.10-0.70         |
| Mn+Ni      | 0.50-2.00         |
| 5 But Mn   | 0.50-1.60         |
| Ni         | 0.03-0.80         |
| Mo         | 0.15-0.70         |
| Cu         | 0.05-0.80         |
| Cr         | 0.03-1.00         |
| 10 Sol. Al | 0.01-0.1          |
| N          | 0.002-0.007       |
| Nb         | 0.005-0.04        |
| B          | 0.0005-0.005      |
| Ti         | 0.005-0.05        |

- 15 The remainder: Fe and unavoidable impurities. The reasons for the limited ranges above mentioned for the constituents of the present invention steel are as follows:
- 20 Carbon is one of the more potent and more economical strengthening elements. It is well known that carbon has the strongest influence upon hardenability of weld zone. Accordingly, it is to be desired that carbon content be low as much as possible. Carbon of more than 0.05%, however, is practical from this point of steel making. The upper limit of carbon content, which is 0.15%, is recommended, owing to the need of making 0.01 to 0.03% Nb solute at a quenching temperature of 900° C. to 1000° C., so as to cause Nb-carbide after tempering treatment.
- 25 Niobium content must be determined in consideration of carbon content. According to our experimentations, it is shown that Nb of more than 0.05% scarcely contributed to strength steel. Also, it is impossible to obtain the required strength when Nb content is less than 0.005%. The suitable Nb content in the present invention consists in the range of 0.005% to 0.05%.
- 30 Manganese of 0.50% which is the lower limit is adopted in consideration of this point of steel making and of hot-workability. Also, 1.60% Mn which is the upper limit is determined in consideration of weldability.
- 35 Up to 0.8% nickel causes toughness of steel to increase and results in economical benefits.
- 40 When copper content is above 0.5%, nickel must be added simultaneously. More than 0.03% chromium possibly causes strength and hardenability of steel to increase.
- 45 0.15% to 0.7% molybdenum possibly causes strength of steel to markedly increase. However, when the content is more than 0.7%, weldability of steel is spoiled and when the content is less than 0.15%, strength of steel is harmed.
- 50 More than 0.1% aluminum decreases cleanliness and spoils weldability of steel. Also less than 0.01% aluminum brings about a bad influence to addition of boron in steel making stage.
- 55 When silicon content is above 0.7% toughness and weldability of steel is harmed.
- 60 Up to 0.7% boron possibly causes hardenability of steel to increase without a bad influence to toughness and workability of steel.
- 65 0.005% to 0.05% titanium is a useful element for improving hardenability of steel and for increasing strength of steel owing to precipitation of Ti-carbide in the tempering treatment stage.
- Nitrogen content has a serious influence on combination of Nb-Ti-B which is the main point in the present invention. By reasons of which nitrogen has powerful affinity

to the above three elements, particularly Ti, the content must be limited within the range in which it is impossible to form its nitride. More than 0.007% nitrogen harms toughness of steel, owing to the formed Ti-nitride and causes Ti-carbide, which is effective for strength of steels to decrease. Nitrogen content of the lower limit is 0.002% according to a restriction of steel making process.

In the range of the above-mentioned chemical composition, the following range is recommended as preferred values:

|        | Percent by weight |
|--------|-------------------|
| C      | 0.06-0.12         |
| Si     | 0.10-0.50         |
| Mn+Ni  | 1.00-0.60         |
| Cu     | 0.20-0.40         |
| Cr     | 0.20-0.60         |
| Mo     | 0.20-0.60         |
| Sol Al | 0.010-0.050       |
| Nb     | 0.005-0.03        |
| Ti     | 0.01-0.03         |
| B      | 0.001-0.005       |
| N      | less than 0.005   |

As mentioned above, the present invention steel is composed of alloying of a small quantity of components, and demonstrates yield strength of more than 70 kg./mm.<sup>2</sup>, superior toughness and excellent weldability according to heat treatment of quenching mother steel from more than 4C<sub>3</sub> temperature and then of tempering at more than 600° C.

The following Table I shows examples of the present invention steel. In Table I from A to G, steels are the present invention steels. And from H to K, which are out of the range of components based on the present invention, these steels are shown in comparison with the present invention steel. L steel is an ordinary high-strength low alloy steel.

Examining the above-mentioned values, it is understood that maximum hardness in taper hardness test is far lower than the maximum value required by the same kind of high strength steel, such as Hv≤430 in Japanese WES Standard. This fact shows that hardness of welding zone is markedly lowered according to keeping yield strength of 70 kg.mm.<sup>2</sup> by means of a suitable combination of Nb+Ti+B and at the same time main alloying elements, such as C, Mn, Ni, Cr, Mo and the like, are far less than ordinary high-strength steels.

As for crack sensitivity, also it is shown that occurrence of some crack in the present invention steels can be completely eliminated on condition of simple pre-heating of 75° C. in comparison with high preheating of 100° C. for ordinary high-strength steel.

Although the present invention has been described in conjunction with preferred examples, it is to be understood that modifications and variations may be resorted to without departing from the spirit and scope of the invention as those skilled in the art will readily understand.

What we claim is:

1. High strength low alloy steels composed of 0.05 to 0.15% C, 0.10 to 0.70% Si, 0.50 to 2.00% Mn+Ni, (but 0.50 to 1.60% Mn, and 0.03 to 0.80% Ni), 0.05 to 0.80% Cu, 0.03 to 1.00% Cr, 0.01 to 0.10% Sol. Al, 0.002 to 0.007% N, 0.005 to 0.04% Nb, 0.0005 to 0.005% B, 0.005 to 0.05% Ti and having a yield strength of more than 70 kg./mm.<sup>2</sup> and possessing sufficient weldability.

2. High strength low alloy steels in accordance with claim 1, in which the alloying ingredients comprise 0.06 to 0.12% C, 0.10 to 0.50% Si, 1.00 to 1.60% Mn+Ni, 0.20 to 0.40% Cu, 0.20 to 0.60% Cr, 0.20 to 0.60% Mo, 0.010 to 0.050% Sol. Al, 0.005 to 0.05% Nb, 0.01 to 0.03 Ti, 0.001 to 0.003% B, up to 0.005% N.

3. High strength low alloy steel in accordance with claim 1, wherein the steel following heat treatment is

TABLE I

| Chemical composition |      |      |      |       |       |      |      |      |      |       |      |       | Chemical compound |             |                               |               |                   |           |                         | Mechanical properties |  |  |  |  |  |  |
|----------------------|------|------|------|-------|-------|------|------|------|------|-------|------|-------|-------------------|-------------|-------------------------------|---------------|-------------------|-----------|-------------------------|-----------------------|--|--|--|--|--|--|
| C                    | Si   | Mn   | P    | S     | Cu    | Ni   | Cr   | Mo   | Nb   | Ti    | B    | Al    | N                 | Yield point | Tensile strength <sup>1</sup> | Elongation, % | vE <sub>0.2</sub> | vTrs, °C. | vTr <sub>15</sub> , °C. |                       |  |  |  |  |  |  |
| A.....               | 0.09 | 0.13 | 1.05 | 0.020 | 0.015 | 0.30 | 0.25 | 0.44 | 0.42 | 0.012 | 0.03 | 0.002 | 0.035             | 0.0051      | 77.1                          | 80.6          | 23.1              | 18.7      | -94                     | <-100                 |  |  |  |  |  |  |
| B.....               | 0.11 | 0.16 | 1.10 | 0.018 | 0.011 | 0.31 | 0.26 | 0.46 | 0.42 | 0.015 | 0.03 | 0.002 | 0.036             | 0.0045      | 75.8                          | 80.2          | 22.5              | 24.3      | -58                     | -93                   |  |  |  |  |  |  |
| C.....               | 0.10 | 0.16 | 1.06 | 0.015 | 0.014 | 0.24 | 0.31 | 0.44 | 0.42 | 0.017 | 0.02 | 0.001 | 0.036             | 0.0035      | 81.2                          | 83.4          | 23.3              | 17.9      | -52                     | -97                   |  |  |  |  |  |  |
| D.....               | 0.10 | 0.21 | 1.24 | 0.014 | 0.014 | 0.24 | 0.27 | 0.46 | 0.42 | 0.021 | 0.02 | 0.003 | 0.048             | 0.0041      | 83.3                          | 85.1          | 23.3              | 16.7      | -60                     | -102                  |  |  |  |  |  |  |
| E.....               | 0.10 | 0.22 | 1.29 | 0.023 | 0.013 | 0.30 | 0.03 | 0.54 | 0.39 | 0.016 | 0.02 | 0.002 | 0.042             | 0.0067      | 78.7                          | 83.2          | 24.8              | 18.9      | -75                     | <-120                 |  |  |  |  |  |  |
| F.....               | 0.10 | 0.20 | 1.23 | 0.022 | 0.007 | 0.27 | 0.03 | 0.57 | 0.38 | 0.015 | 0.01 | 0.002 | 0.042             | 0.0065      | 78.7                          | 83.1          | 23.6              | 19.2      | -74                     | -111                  |  |  |  |  |  |  |
| G.....               | 0.12 | 0.17 | 1.24 | 0.022 | 0.016 | 0.30 | 0.03 | 0.53 | 0.39 | 0.033 | 0.02 | 0.002 | 0.062             | 0.0062      | 79.0                          | 83.1          | 23.9              | 14.9      | -42                     | -73                   |  |  |  |  |  |  |
| H.....               | 0.10 | 0.13 | 1.16 | 0.020 | 0.019 | 0.39 | 0.27 | 0.44 | 0.40 | 0.012 | 0.03 | 0.002 | 0.040             | 0.0112      | 70.7                          | 75.8          | 23.9              | 10.9      | -7                      | -45                   |  |  |  |  |  |  |
| I.....               | 0.10 | 0.24 | 1.27 | 0.021 | 0.017 | 0.28 | 0.03 | 0.57 | 0.39 | Tr.   | 0.02 | 0.002 | 0.050             | 0.0084      | 65.1                          | 72.6          | 28.0              | 21.5      | -103                    | <-120                 |  |  |  |  |  |  |
| J.....               | 0.10 | 0.20 | 1.26 | 0.021 | 0.013 | 0.28 | 0.04 | 0.53 | 0.39 | 0.016 | 0.06 | 0.002 | 0.039             | 0.0069      | 77.7                          | 82.9          | 24.5              | 11.0      | -18                     | -58                   |  |  |  |  |  |  |
| K.....               | 0.12 | 0.23 | 1.30 | 0.023 | 0.015 | 0.38 | 0.26 | 0.48 | 0.40 | 0.015 | Tr.  | 0.002 | 0.028             | 0.0116      | 69.3                          | 75.2          | 20.7              | 23.9      | -72                     | <-100                 |  |  |  |  |  |  |
| L.....               | 0.12 | 0.26 | 0.86 | 0.016 | 0.018 | 0.27 | 0.85 | 0.53 | 0.54 | V0.05 | Tr.  | 0.004 | 0.028             | 0.0065      | 77.1                          | 83.0          | 23.5              | 11.3      | -89                     | -104                  |  |  |  |  |  |  |

<sup>1</sup> Kg./mm.<sup>2</sup>. <sup>2</sup> Kgm./cm.<sup>2</sup>.

In Table II, the values of which hardness and crack sensitivity of B, C, D and L steels in Table I are tested by means of both taper hardness test and y-type slit crack test methods are shown.

quenched at a temperature from AC<sub>3</sub> to 1050° C. and then is tempered at less than AC<sub>1</sub> temperature.

4. High strength low alloy steel in accordance with claim 2, wherein the steel following heat treatment is

TABLE II

| Maximum hardness in taper hardness test at 28° C./sec. (Hv) | Pre-heating at 75° C. |                     |                   | Pre-heating at 100° C. |                     |                   |
|-------------------------------------------------------------|-----------------------|---------------------|-------------------|------------------------|---------------------|-------------------|
|                                                             | Surface crack ratio   | Section crack ratio | Route crack ratio | Surface crack ratio    | Section crack ratio | Route crack ratio |
| B.....                                                      | 370                   | 0                   | 0                 | 0                      | 0                   | 0                 |
| C.....                                                      | 360                   | 0                   | 0                 | 0                      | 0                   | 0                 |
| D.....                                                      | 365                   | 0                   | 0                 | 0                      | 0                   | 0                 |
| L.....                                                      | 405                   | 5                   | 20                | 40                     | 0                   | 0                 |

3,592,633

5

quenched at a temperature from  $AC_3$  to  $1050^{\circ}$  C. and  
then is tempered at less than  $AC_1$  temperature.

6

3,368,887 2/1968 Clark ----- 75-128R

HYLAND BIZOT, Primary Examiner

References Cited

UNITED STATES PATENTS

5

U.S. CL. X.R.

2,750,283 6/1956 Loveless ----- 75-124  
3,216,823 11/1965 Gulya ----- 75-124  
5 75-125, 128R; 148-31

UNITED STATES PATENT OFFICE  
CERTIFICATE OF CORRECTION

Patent No. 3,592,633 Dated July 13, 1971  
Inventor(s) TATSUMI OSUKA et al

It is certified that error appears in the above-identified patent  
and that said Letters Patent are hereby corrected as shown below:

Column 4, line 24 (Claim 1, line 3) - before "0.05"  
insert "0.15 to 0.70% Mo".

Signed and sealed this 15th day of February 1972.

(SEAL)

Attest:

EDWARD M.FLETCHER, JR.  
Attesting Officer

ROBERT GOTTSCHALK  
Commissioner of Patents